

## UNITED STATES PATENT OFFICE

2,160,406

PRODUCT FOR INHIBITING THE ATTACK  
ON METALS BY ACIDS OR SALTS AND ITS  
APPLICATIONSJacques Edouard Julien Georges Mascré,  
Premery, France, assignor to Etablissements  
Lambiotte Frères Premery (Nièvre), France, a  
corporation of FranceNo Drawing. Application November 17, 1936,  
Serial No. 111,336. In France December 17,  
1935

6 Claims. (Cl. 148—8)

It is known that metals are attacked by acids in the absence of oxygen under conditions which depend both upon the nature of the metal and upon that of the acid.

5 In principle for a given acid the attack is more rapid, that is to say the dissolution is more rapid, if the metal is situated lower in the scale of solution pressures, the corresponding evolution of hydrogen being more ready.

10 It is likewise known that certain substances oppose this evolution of hydrogen and thus render the metal passive. Arsenious anhydride, formaldehyde, aniline and pyridine manifest this tendency to degrees which vary greatly according to the case. In fact certain bodies like arsenious anhydride and Formol behave sometimes as inhibitors and sometimes as accelerators of the attack on metals by acids.

Now according to the present invention it 20 has been observed the oils obtained in the carbonization of wood have a very much greater inhibiting power for equal weight of the product employed, than that of all known compositions and an efficaciousness which is quite general in all cases.

It is known that in the carbonization of wood a pyroligneous liquid is obtained which by distillation gives crude wood spirit which contains besides methanol, methyl acetate, acetone and allyl alcohol, a fraction of oils which will be referred to as "crude wood spirit oils", which may be separated either by rectification or by dilution of the crude wood spirit with water.

These oils have a density between 0.890 and 35 0.935, most generally 0.910 to 0.925. They distil from 50—220° C. 80—90% passing on the average from 120—130° C. to 205—210° C. They are rich in ketonic products (30—45% calculated as acetone) and allyl compounds (10—30% calculated 40 as allyl alcohol).

To sum up, these oils contain ketones, aldehydes, diketones, alcohols, hydrocarbons, furane and cyclopentane derivatives, amines, and other products which are unknown or not identified 45 at present but which contribute for their part to the special and characteristic properties of these oils.

According to the present invention the unexpected discovery has been made that these oils 50 and all the fractions which are still very complex and which can be separated therefrom in one way or another exhibit inhibitory properties towards the attack on metals by acids or strongly dissociated salts.

55 They may thus be very usefully employed for

preventing if not entirely at least almost entirely attack on a metal whenever the latter is put into contact with an acid or a salt which attacks it. This is particularly the case with cleaning, pickling, or treatment of metals by acids, and in the case of scaling metallic surfaces by acids. It is sufficient to mix the oils with the pickling or scaling baths used, and their presence in these baths does not at all alter the solubility in the acid of the oxide or scale. It should likewise be added that their wetting power facilitates their action and renders it regular.

But though these crude wood oils may be used for this purpose they have the disadvantage of not being entirely soluble in aqueous solutions of acids and of consequently giving rise to a greater or less degree to blackish tars which are deposited upon the walls of the receptacles.

To remedy this disadvantage it has been observed that it is sufficient to destroy by resinifying the unstable components of the oils, for example by bringing them to boiling in an acid medium, then in extracting from the oils thus treated the active, soluble and stable products with the aid of aqueous solutions of acids or with the aid of pure water, and to utilise these extracts either as such or if necessary in deodorized form.

By way of non-limiting example of the manufacture of extracts of crude wood spirit oils one 30 may operate as follows:

To 1 part by volume of crude wood spirit oils is added 1 part by volume of 7% hydrochloric acid or 10% sulphuric acid. The mixture is brought to boiling under a reflux for 10 hours.

After cooling the lower aqueous layer representing 1.05 to 1.10 parts by volume is decanted, clarified, and constitutes a stable extract containing 7—10% of dissolved active crude wood spirit oils.

The residual oil about 0.9 part by volume may be extracted again by agitation in the cold with an equal volume of acid as described above and give a new quantity of extract only half as rich as the above extract.

Thus systematic extractions may be combined on this principle.

A practically deodorized extract may be obtained by eliminating from the above extracts by distillation with a column, a first fraction of 10% which entrains the most volatile and strongly odoriferous constituents.

This distilled fraction constitutes moreover a stable and soluble very strongly active extract.

In the following there are given a certain number of results of experiments with extracts of wood oils mixed with baths for pickling or scaling.

1. Pickling baths.

The tests were effected upon portions of drawn iron tube and pickled and cleaned.

|                                                                                                                       | The weight losses per square meter per hour were for an average duration of— |           |  |
|-----------------------------------------------------------------------------------------------------------------------|------------------------------------------------------------------------------|-----------|--|
|                                                                                                                       | 50 hours                                                                     | 250 hours |  |
| <i>(a) Treatment in the cold (20° C.) with a solution of pure hydrochloric acid with 23 grams of HCl per 100 ccs.</i> |                                                                              |           |  |
| Pure hydrochloric acid alone                                                                                          | 389                                                                          | -----     |  |
| Pure hydrochloric acid+1% arsenious anhydride                                                                         | 332                                                                          | -----     |  |
| Pure hydrochloric acid+1% of aniline                                                                                  | 179                                                                          | -----     |  |
| Pure hydrochloric acid+5% of formol (30%)                                                                             | 6.17                                                                         | 8.02      |  |
| Pure hydrochloric acid+1% of crude wood oils                                                                          | 2.09                                                                         | 8.62      |  |
| Pure hydrochloric acid+10% of a 6-9% sulphuric acid extract of dissolved wood oils                                    | 2.80                                                                         | 4.13      |  |
| Pure hydrochloric acid+10% of a 7-10% hydrochloric acid extract of dissolved wood oils                                | 2.25                                                                         | 3.43      |  |
| <i>(b) Treatment in the cold (20° C.) with a solution of pure sulphuric acid with 30.6 grams per 100 ccs.</i>         |                                                                              |           |  |
| Pure sulphuric acid alone                                                                                             | 262                                                                          | -----     |  |
| Pure sulphuric acid+1% of aniline                                                                                     | 155                                                                          | -----     |  |
| Pure sulphuric acid+1% of formol (30%)                                                                                | 5.37                                                                         | 4.75      |  |
| Pure sulphuric acid saturated with arsenious anhydride                                                                | 0.792                                                                        | 1.31      |  |
| Pure sulphuric acid+10% of a 6-8% sulphuric acid extract of dissolved wood oils                                       | 0.540                                                                        | 0.615     |  |
| Pure sulphuric acid+10% of a 3-6% deodorised sulphuric acid extract of dissolved wood oils                            | 0.885                                                                        | 1.87      |  |
| <i>(c) Hot treatment (60° C.) with a solution of pure sulphuric acid with 21.91 grams per 100 ccs.</i>                |                                                                              |           |  |
| Pure sulphuric acid alone                                                                                             | 1030                                                                         | -----     |  |
| Pure sulphuric acid+1% aniline                                                                                        | 843                                                                          | -----     |  |
| Pure sulphuric acid+1% formol (30%)                                                                                   | 107                                                                          | -----     |  |
| Pure sulphuric acid+10% of a 6-9% sulphuric acid extract of dissolved wood oils                                       | 28                                                                           | -----     |  |
| Pure sulphuric acid+10% of a 3-6% sulphuric acid extract of dissolved wood oils                                       | 77                                                                           | -----     |  |

2. Scaling baths.

The scaling solutions employed all contained 3.5 grams of gaseous HCl per 100 ccs.

| 5                                                                                     | The weight losses in grams per square meter per hour were for an average duration of— |           |  |
|---------------------------------------------------------------------------------------|---------------------------------------------------------------------------------------|-----------|--|
|                                                                                       | 24 hours                                                                              | 100 hours |  |
| <i>(a) Upon portions of drawn iron tube pickled and cleaned</i>                       |                                                                                       |           |  |
| Pure hydrochloric acid alone                                                          | 78.2                                                                                  | -----     |  |
| Water+10% of commercial scaling compound with a basis of arsenious anhydride          | 2.80                                                                                  | 6.0       |  |
| Water+10% of commercial scaling compound with a basis of formol                       | 0.405                                                                                 | 0.602     |  |
| Pure hydrochloric acid+1% of a 7-10% hydrochloric acid extract of dissolved wood oils | 0.501                                                                                 | 0.803     |  |

The weight losses in grams per square meter per hour were for an average duration of— 5

| (b) Upon crude sheet of pure aluminum for industrial apparatus                          | 24 hours | 48 hours | 10 |
|-----------------------------------------------------------------------------------------|----------|----------|----|
|                                                                                         | 3.99     | 4.68     |    |
| Pure hydrochloric acid alone                                                            | 5.88     | 17.4     |    |
| Water+10% commercial scaling compound with a basis of arsenious anhydride               | 27.2     | 13.4     |    |
| Water+10% of a commercial scaling compound with a basis of formol                       | 10.6     | 11.4     | 15 |
| Pure hydrochloric acid+1% of formol (30%)                                               | 0.89     | 0.96     |    |
| Pure hydrochloric acid+1% of a 7-10% hydrochloric acid extract of dissolved wood oils   | 0.28     | 0.17     |    |
| (c) Upon crude zinc sheet                                                               |          | 2 hours  | 20 |
| Pure hydrochloric acid alone                                                            | 800      | -----    |    |
| Water+10% of commercial scaling compound with a basis of arsenious anhydride            | 2070     | -----    |    |
| Water+10% commercial scaling compound with basis of formol                              | 930      | -----    |    |
| Pure hydrochloric acid+1% formol (30%)                                                  | 900      | -----    | 15 |
| Pure hydrochloric acid+10% of a 10-18% hydrochloric acid extract of dissolved wood oils | 0.74     | 0.29     |    |

For pickling and scaling baths the results are substantially the same with the ordinary acids of commerce more or less charged with impurities. 30

It has moreover been observed that even in the presence of accelerating impurities like arsenious anhydride the wood oils or their extracts maintain practically the whole of their efficiency. 35

What I claim is:

1. A metal treating bath comprising a diluted mineral acid and as an inhibitor product preventing the attack of the metal itself a low proportion of crude wood spirit oils arising from the carbonization of wood. 40

2. A metal pickling bath comprising a diluted mineral acid and as an inhibitor product preventing the attack of the metal itself a low proportion of crude wood spirit oils arising from the carbonization of wood. 45

3. A metal scaling bath comprising a diluted mineral acid and as an inhibitor product preventing the attack of the metal itself a low proportion of crude wood spirit oils arising from carbonization of wood. 50

4. A metal treating bath comprising diluted hydrochloric acid and as an inhibitor product preventing the attack of the metal itself a low proportion of crude wood spirit oils arising from the carbonization of wood. 55

5. A metal treating bath comprising diluted sulphuric acid and as an inhibitor product preventing the attack of the metal itself a low proportion of crude wood spirit oils arising from the carbonization of wood. 60

6. A metal treating bath comprising a diluted mineral acid and as an inhibitor product preventing the attack of the metal itself a low proportion of an aqueous extract of wood spirit oils. 65

JACQUES EDOUARD JULIEN

GEORGES MASCRÉ